

## 1

2,899,388

### CALCIUM BASE GREASE CONTAINING A NICKEL, LEAD OR LITHIUM SALT OF A DIALKYL DITHIOPHOSPHORIC ACID DIESTER

John Walter Nelson, Lansing, and Milton P. Kleinholz, Homewood, Ill., assignors to Sinclair Refining Company, New York, N.Y., a corporation of Maine

No Drawing. Application February 6, 1957  
Serial No. 638,476

#### 2 Claims. (Cl. 252—32.7)

This invention relates to soap-thickened greases which are inhibited against oxidation. More particularly, this invention provides for the inhibition of anhydrous calcium 12-hydroxy stearate greases by the incorporation of certain oil-soluble metal salts of diester dithiophosphates.

It is generally known that certain of the metal salts of the diesters of dithiophosphoric acids impart desirable properties to mineral lubricating oils when added in minor amounts. Particularly, these salts afford increased resistance to oil oxidation and bearing corrosion as evidenced by Patent No. 2,364,283 to Freuler. However, the prior art has not generally made a distinction between the use of these additives in greases and fluid lubricating oils nor between the different types of grease-metal-salt combinations but apparently has acted upon the assumption that a metal diester dithiophosphate showing improved oxidation inhibiting characteristics in one lubricating oil or grease will give substantially the same result when used in other lubricating oils or greases.

The problems concerned with the inhibition of oxidation in a fluid lubricating oil are normally different from the inhibition of oxidation in a solid lubricating grease in that the grease is subjected to much higher stresses and localized temperatures next to bearing surfaces which increases the tendency for oxidizing the base oil, such oxidation often being catalyzed by the thickening soap. Furthermore, among the various grease compositions there is found different so-called gel structures in each grease and subsequently unique problems existing in relation to each grease. Moreover, the soap used in thickening one type of grease composition may be more prone to deterioration than the soap used in thickening another type of grease composition and even if the two soaps are prone to deterioration in the same degree it has been found that the different metallic substituents used in the soaps can catalyze the oxidation of the oil component to varying extents. Thus, it has become highly important to learn as much as possible about the effect of each of the oxidation inhibiting agents in different soap thickened greases and to establish some definite correlation between the inhibiting agents and particular greases.

According to this invention, we have found that certain of the metal salts of the diesters of dithiophosphoric acids while known to act generally as oxidation inhibiting agents in fluid lubricating oils, do not give uniformly good results when added to dissimilar soap thickened greases.

## 2

Whether this can be attributed to the catalytic effect of the metals of the different metallic soap thickening agents or to the inherently different gel structures of the greases or to other causes is unknown at the present time. More particularly, we have found that about 0.1 to 5.0% and preferably about 0.5 to 2.0% by weight of the oil-soluble nickel, lead and lithium salts of dialkyl dithiophosphoric acid diesters show excellent oxidation inhibiting characteristics when added to anhydrous calcium 12-hydroxy stearate grease while little, if any, improvement of the oxidation inhibiting characteristics are realized if the same salts in the same proportions are used in a lithium 12-hydroxy stearate grease. Moreover, these nickel, lead and lithium salts in the above amounts are more effective in inhibiting the oxidative tendencies of anhydrous calcium 12-hydroxy stearate greases than many of the other phosphoric acid ester salts such as barium, zinc or vanadium dialkyl dithiophosphates or other commercially recognized oxidation inhibitors such as Ortholeum 300 (primarily a diphenylamine).

The metal salts of the diester dithiophosphate can be prepared by any of the well-known processes, such as by reacting an alcohol with phosphorous pentasulfide to form a di-substituted sulfur containing phosphoric acid and subsequently neutralizing the acid with a metal oxide, hydroxide or carbonate. The organic substituents of the acid can be any alkyl of four to twelve carbon atoms, e.g. eight, providing the metal salts have sufficient oil solubility to afford the desired oxidation inhibiting properties. Advantageously, the total number of carbon atoms in the two alkyl groups of the diesters will be about 12 to 18. Examples of useful alcohols are, 2-methylpentanol-1, decanol, hexanol, heptanol, 2-ethylhexanol, etc. In addition, mixtures of the alcohols can be utilized if desired.

The effectiveness of various diester metal salts were evaluated in an anhydrous calcium 12-hydroxy stearate and a lithium 12-hydroxy stearate grease. These greases were comprised of a mineral base oil of lubricating viscosity, e.g. about 50 SUS at 100° F. to 200 SUS at 210° F., thickened to grease consistency with calcium or lithium 12-hydroxy stearate. Usually the soap will be about 4 to 30% by weight of the total grease composition and can be made from any fatty source such as the corresponding acid ester or glyceride. The salts evaluated were the nickel, lithium, lead, barium, zinc and vanadium salts of di-(2-ethylhexyl)-dithiophosphoric acid.

The anhydrous calcium 12-hydroxy stearate greases which are to be inhibited by our preferred salts can be prepared by any of the conventional methods, the following being but an illustrative example. The greases can contain various additive components other than the antioxidant, such as the corrosion inhibitors, etc. Usually, in commercial procedures, the additives are incorporated before milling.

#### Example I

Twenty pounds of 12-hydroxy stearic acid, 10 pounds of water, and sixty pounds of mineral oil containing 2.9 pounds of hydrated lime previously slurried in part of this oil were mixed in a steam heated kettle at 100° F. The mineral oil used was an 82 SUS/100° F. blend of

80 volume percent solvent treated Mid-Continent neutral and 20 volume percent conventionally refined naphthenic base Coastal stock. The temperature was raised gradually and at about 130° F. a pronounced thickening occurred indicating reaction. The initial formation of a smooth soap took place in the heterogeneous phase system at a temperature well below the melting point of the acid, i.e., below about 160° F., as indicated by presence of a few solid acid flakes on the kettle walls where temperature was maximum. During formation of the smooth, homogeneously thickened mass in the temperature range 130 to 190° F. free water was rejected, appearing at the surface and edge of the reaction mass in the kettle. The separated free water changed from cloudy to clear, showing essentially complete reaction of the lime and acid. The temperature was raised from 190° F. to 225° F. to evaporate visible non-emulsified water in order to preclude later foaming. An additional five parts of the oil blend (based on weight of fatty acid employed) was incorporated while raising the temperature from 225 to 240° F. Dehydration in the temperature range of 225 to 240° F. was accompanied by gradual, smooth gel formation. The temperature was then raised to about 250 to 255° F. and held one hour to insure complete dehydration after which the grease was cooled to 170° F. while incorporating the remainder of the oil (90 pounds). The grease was then milled at 170° F., 0.005 inch clearance and a flow rate of 1.5 pounds per minute in a conventional colloid mill.

In these evaluation tests, the anhydrous calcium 12-hydroxy stearate grease was prepared essentially as described in Example I having 10.8% by weight calcium 12-hydroxy stearate incorporated therein. The lithium 12-hydroxy stearate greases used in these tests were prepared by charging the fatty component, the lithium base and a portion of the mineral lubricating oil base into a steam jacketed grease kettle and thoroughly mixing at 180° to 190° F. until saponification was substantially complete. The resulting soap concentrate was dehydrated at 300° to 320° F. After dehydration the heat was shut off and the remainder of the mineral lubricating oil base was blended with the soap concentrate. The constituents were proportioned so as to give about 10.4% by weight of the lithium 12-hydroxy stearate in the final grease composition.

Both of the above greases were milled once on a Charlotte colloid mill, weighed into one-pound cans and heated overnight at 200° F. 1.0 percent by weight of each of the metal salts was weighed directly into the separate grease cans and the mixtures stirred with a motor driven stirrer until the salt was blended throughout the mixture. 1.0 percent by weight of Ortholeum 300, a well-known commercial oxidation inhibiting agent, containing a mixture of alkylphenylamines, principally diphenylamine was blended with each of the greases and used as a reference blend. The samples were tested by the Norman-Hoffman oxidation test regular method (ASTM D-942-50) and the more severe bronze block method. These tests were terminated when the oxygen pressure dropped 55 pounds or after a run of 500 hours. The following table gives pertinent data relative to these grease compositions.

| Metal of Salt      | Lithium 12 Hydroxy Stearate Grease, Lbs. Pressure Drop/Hours |              | Anhydrous Calcium 12 Hydroxy Stearate Grease, Lbs. Pressure Drop/Hours |              |
|--------------------|--------------------------------------------------------------|--------------|------------------------------------------------------------------------|--------------|
|                    | Regular                                                      | Bronze Block | Regular                                                                | Bronze Block |
| Zn.....            | 35/500                                                       | 55/118       | 34/500                                                                 | 55/334       |
| Ni.....            | 48/500                                                       | 55/174       | 6/500                                                                  | 6/500        |
| Pb.....            | 16/500                                                       | 55/132       | 6/500                                                                  | 4/500        |
| Ba.....            | 46/500                                                       | 55/120       | 55/380                                                                 | 55/442       |
| Li.....            | 55/105                                                       | 55/77        | 7/500                                                                  | 6/500        |
| Va.....            | 55/24                                                        | 55/55        | 55/38                                                                  | 55/42        |
| None.....          | 22/500                                                       | 55/82        | 55/50                                                                  | 55/31        |
| Ortholeum 300..... | 16/500                                                       | 36/500       | 10/500                                                                 | 11/500       |

From the above table, it will be noted that the nickel, lead and lithium salts of di-(2-ethylhexyl)-dithiophosphate show a very pronounced improvement over the other metal salts of the same dithiophosphate in respect to the oxidation characteristics in both the regular method and the bronze block method and a substantial improvement over the commercial inhibiting agent when incorporated in an anhydrous calcium 12-hydroxy stearate grease. Comparing the results obtained in the anhydrous calcium 12-hydroxy stearate grease with those obtained in the lithium 12-hydroxy stearate grease, a substantially different effect is immediately noticed. None of the salts displayed any substantial oxidation inhibition in the bronze block method and thus were essentially useless in comparison with the commercial product while the lead salt was the only one which showed any oxidation inhibition in the regular method, this being no substantial improvement over the commercial product. All of the other salts were inferior to the uninhibited sample or to the commercial product and in some instances apparently promoted oxidation.

It is evident from an examination of this data that the selection of the proper metal dithiophosphate oxidation inhibiting agent depends both upon the type of grease utilized and the particular metal salt employed and that these may not be indiscriminately chosen if uniformly good results are to be obtained.

We claim:

1. A lubricating grease composition consisting essentially of a major portion of a base mineral lubricating oil thickened to grease consistency with anhydrous calcium 12-hydroxy stearate and about 0.1 to 5.0% by weight of an oil-soluble metal salt of a dialkyl dithiophosphoric acid diester, said alkyl groups containing about 4 to 12 carbon atoms, and the metal of said salt being selected from the group consisting of nickel, lead and lithium.

2. The lubricating grease composition of claim 1 where-in the oil-soluble metal salt of the dialkyl diester of the dithiophosphoric acid is present in amounts of about 0.5 to 2% by weight.

#### References Cited in the file of this patent

#### UNITED STATES PATENTS

- 2,364,283 Freuler \_\_\_\_\_ Dec. 5, 1944  
 2,607,734 Sproule et al. \_\_\_\_\_ Aug. 19, 1952